# EUROPEAN PATENT SPECIFICATION

(11) **EP 0 353 013 B1**
(45) Date of publication and mention of the grant of the patent: **15.09.1993**
(21) Application number: 89307524.2
(22) Date of filing: 25.07.1989
(51) Int. Cl.: A47L 13/17, C11D 17/04

(54) **Wiping article**
Wischgegenstand
Article d'essuyage

(30) Priority: 26.07.1988 GB 8817728
(43) Date of publication of application: 31.01.1990
(73) Proprietor: UNILEVER PLC, London EC4P 4BQ (GB); UNILEVER N.V., 3013 AL Rotterdam (NL)
(72) Inventor: Edwards, Keith Andrew, Wirral Merseyside L63 5JT (GB); Leng, Christine Ann, Wirral Merseyside (GB); Sams, Philip John, Willaston South Wirral LL4 1TB (GB)
(74) Representative: Ford, Michael Frederick

(56) References cited:
- EP-A- 0 161 911
- EP-A- 0 273 467
- FR-A- 2 353 265
- US-A- 3 949 137

## Description

The invention relates to a wiping article suitable for use in cleaning soiled surfaces in the presence of water. The wiping article can be adapted for cleaning hard surfaces, particularly those to be found in the domestic kitchen and bathroom, or for cleaning the surface of the human body, for instance when taking a shower.

There have been a number of prior proposals for impregnated wiping articles for hard surfaces e.g. DE-C-2625176 (Schickedanz), EP-A-66463 (Unilever) and EP-A-211664 (Unilever). There have also been prior proposals for impregnated "cloths" for washing the human body surface, e.g. EP-A-68516 (Barbey & Hecken) and US-A-4303543 (Procter & Gamble). EP-A-161911 (Unilever) is relevant to both applications.

It has been proposed, e.g. in the above-mentioned EP-A-66463 and EP-A-211664 and in EP-A-273467, to provide a hard surface wiping article as a sandwich structure with first and second substrate layers sandwiching a core of concentrated surfactant.

A problem which can arise with both the above-mentioned categories of wiping article is that when used in the presence of a substantial quantity of water the soap or detergent active with which they are impregnated is leached out too quickly, leaving the article prematurely exhausted of soap or detergent active. This might for instance be manifested as a hard surface wipe being exhausted after a single use, or a wipe intended for use under the shower failing to complete a single use.

EP-A-161911 proposed to delay release of impregnating detergent active compound by means of moisture barrier areas, applied in a pattern to sandwich the detergent active applied in a similar pattern and retarding the leaching of the detergent active from the wipe.

Our EP-A-211664, mentioned above, proposed a wiping article for hard surfaces in which surfactant was trapped in a polymeric matrix material, thereby conferring controlled release properties.

We have now found that release of surfactant can be retarded in a simpler way.

According to the present invention there is provided a substantially dry-to-the-touch wiping article which is suitable for use in cleaning soiled surfaces in the presence of water,
the article comprising first and second substrate layers with surfactant in solid form sandwiched between them,
characterised in that the surfactant
i) forms a liquid crystalline phase in contact with water at temperatures above its Krafft temperature and up to at least 30°C, and/or
ii) has a Krafft temperature above 20°C.

Use of a surfactant with a Krafft temperature above 20°C (which is a relatively high Krafft temperature) has the consequence that the surfactant will have poor solubility, and be slow to dissolve, when contacted by water at temperatures up to about the Krafft temperature. This can provide slow release of surfactant when the wiping article is used with cold or lukewarm water.

Preferable, however is formation of a liquid crystal phase when the surfactant comes into contact with water, especially formation of a cubic or hexagonal, most preferably hexagonal, liquid crystal phase. Such liquid crystal phase(s) will form at appropriate points in the concentration gradient between surfactant in the wiping article, and water permeating into the article. Formation of a hexagonal liquid crystal phase when water contacts the solid surfactant is particularly effective in delaying release of surfactant from the wiping article because the liquid crystal phase is highly viscous and is itself slow to dissolve in water, moreover it forms a temporary shield between the remaining solid surfactant and any water.

Formation of a liquid crystal phase will serve to retard dissolution when the wiping article is contacted by water at any temperature at which the liquid crystal phase exists. Desirably this is from 20°C or the surfactant's Krafft temperature (whichever is greater) upwards to at least 30°C, preferably 35 or 40°C, and still better up to 50°C which is approximately the highest temperature which hands can bear. Thus, for forms of the invention in which a liquid crystal phase serves to retard dissolution, either the surfactant will display a Krafft temperature below 20°C with liquid crystal phase existing over a range of temperatures extending at least from 20°C to 30°C, or the surfactant will display a Krafft temperature above 20°C with liquid crystal phase existing over a range of temperatures extending upwards from the Krafft temperature and reaching a temperature which is at least 30°C.

It is important that the surfactant should foam in water, because this provides the user with visual confirmation of the presence of surfactant. For a surfactant with a fairly high Krafft temperature, a fairly high critical micelle concentration would be desirable in order that the surfactant should foam. It is preferred that the critical micelle concentration should be at least 2mMole/litre, better at least 4 or 5mMole/litre.

The surfactant needs to be in the form of a solid, so that it remains in place within the wiping article, when the article is dry.

It is strongly preferred that the surfactant itself can exist as a solid at 20°C, preferably at temperature up to at least 25°C. This makes it possible to incorporate solid concentrated surfactant between the two layers of substrate, and have the surfactant stay in place during storage of the dry wiping article before use. Preferably the solid surfactant should not be sticky, more preferable is that the surfactant is able to exist as dry particles at 20°C, preferably at temperatures of at least 25°C. The surfactant may well be used in particulate form, with the particles trapped between the two substrate layers.

If the surfactant is used in particulate form, then the rate of dissolution may be adjusted to some extent by choice of the size of the surfactant particles.

The surfactant may be a non-soap detergent. Several types can be used. One possible type of surfactant is C₁₄ to C₁₆ sulphobetaines. These readily form hexagonal liquid crystal phases on contact with water. When dry they are crystalline solids.

Preferred surfactants for this invention are mild to the skin, e.g. monoalkyl sulphosuccinates or fatty acyl isethionates where the alkyl or acyl group has from 8 to 22 carbon atoms, preferably 10 to 16 carbon atoms. This anionic surfactant must have a solubilising cation, and alkali metal ions are preferred. In their commercially available forms, these types of surfactant frequently contain fatty acids and other impurities, but this does not reduce their usefulness in the present application.

Particularly preferred is sodium cocoyl isethionate which has a Krafft temperature of 26°C. Above the Krafft temperature both hexagonal and lamella liquid crystal phases form in the concentration gradient between the surfactant and water. When this surfactant is used, at temperatures below the Krafft temperature, there is restricted solubility in water and hence slow rate of dissolution. Above the Krafft temperature the hexagonal liquid crystal phases retards solution. The hexagonal liquid crystal phase exists from the Krafft temperature up to well over 50°C.

As indicated above the invention requires substrate layers. It is substrate layers which provide the wiping surfaces, and which give the article its strength and integrity.

The material of at least one substrate layer must be water permeable. Preferably the substrate layers are sheets of fibrous material.

Particularly preferred is a non-woven fibrous sheet. Cellulose fibres are particularly suitable in view of their ability rapidly to absorb water when employed to clean a soiled surface.

The substrate layers can also comprise other fibrous materials such as polyamide, polyester and polypropylene, or mixtures of such fibres, which are particularly useful in providing the article with extra wet strength.

The wet strength of substrate layer material can also be increased by incorporation of suitable binders such as styrene butadiene lattices, or an acrylic binder, or polyvinyl acetate, or polymer emulsions.

The absorbent substrate can be made from paper, in which case it will generally comprise cellulose fibres which are relatively short in length. Additives, such as hydroxyethyl cellulose may be employed to provide added wet strength.

The substrate layers may be the same or may be different. It can be advantageous to employ different substrate layers, for example choosing one substrate material to provide good wet strength and another substrate material to provide good absorbency. One preferred substrate material is a non-woven comprising cellulose fibres an example of which is Mitsubishi® TCF 408, a 100% cuprammonium rayon spun bonded non-woven having the following technical specifications:

| | |
|---|---|
| Nominal basis weight (g/m²) | 82.5 |
| Thickness (µm) | 500 |
| Dry tensile strength: machine direction (N/m) | 635 |
| Dry tensile strength: cross direction (N/m) | 565 |
| Wet tensile strength: machine direction | 498 |
| Wet tensile strength: cross direction (N/m) | 447 |
| Absorption capacity (g/g) | 5 |

Another substrate material is a non-woven comprising cellulose fibres such as Storalene® 715:50 or Storalene® 717:50 available from Stora-Kopparberg, Sweden, which contains the following ingredients:

The relevant technical specification of Storalene® 715:50 and Storalene® 717;50 are set out below:

| | Storalene | |
|---|---|---|
| | 715:50 | 717:50 |
| Nominal basis weight (g/m²) | 50 | 50 |
| Thickness (µm) | 400 | 365 |
| Dry tensile strength-machine direction (N/m) | 600 | 625 |
| Dry tensile strength-cross direction (N/m) | 450 | 330 |
| Wet tensile strength-machine direction (N/m) | 300 | 205 |
| Wet tensile strength-cross direction (N/m) | 250 | 95 |
| Absorption capacity (g/g) | 4 | 4 |

A further example of a suitable substrate material is Hi-Loft® 3051 available from Scott Paper Co, a random wet-laid lofty paper web having a base weight of 82 g/m² and a porosity of 92%. This is bulky high-porosity sheet material having a high wicking rate.

It is possible for a substrate layer to consist of a laminate of more than one layer, for example a laminate of an absorbent material with a reinforcing material at the exterior surface. It is possible for abrasive particles to be applied to the exterior surface of one or both substrate layers. Suitable abrasive particles are polyvinyl chloride granules. The application of abrasive granules to the exterior surface of a wiping article is described in our published European application EP 211664.

Abrasive material may be applied to the exteriors of both substrate layers, and possibly different abrasive materials could be employed so that one substrate layer provided a harsher abrasive surface than the other. Preferable however is to have abrasive on one substrate layer and a smooth surface on the other substrate layer making it suitable for polishing off after initial cleaning with the abrasive side of the wiping article.

Joining two substrate layers with surfactant sandwiched between them may be accomplished in various ways. It may be carried out by heat sealing the two layers to each other with a regular pattern or array of heat sealing, as described for instance in EP-A-66463 and EP-A-112654. Alternatively the substrate layers may be joined by use of sintered polyethylene in the manner described in our copending application EP-A-353014 filed simultaneously with this application and claiming priority from British application 8817727.4.

### Examples

In these Examples, wiping articles were prepared by a standard procedure, in which particles of surfactant were sandwiched between substrate layers. One substrate layer consisted of Mitsubishi® TCF 408 mentioned above and the other consisted of Hi-Loft® 3051 also mentioned above. To manufacture the wiping article, squares of each substrate material, 30cm along each side were employed. 2.5g polyethylene beads of maximum size 0.3mm were sprinkled over one surface of each square of substrate and the substrate then heated in an oven to melt the beads sufficiently to bond to the substrate layer. A portion of powdered surfactant was then sprinkled over a 27.5cm x 27.5cm portion of the polyethylene-coated surface of one substrate layer, the other substrate layer was then superimposed so that the polyethylene-coated surfaces were confronting each other and sandwiching the surfactant. Then the assembly was passed between heated rollers to effect heat-sealing between the polyethylene layers. The resulting laminate was then trimmed to a square of 28cm along each side.

In this fashion wiping articles were prepared using several surfactant materials and several dosages of each surfactant material. The surfactants employed in these Examples were:
sodium dodecyl sulphate whose Krafft temperature and critical micelle concentration are reported as 16°C and 8mMoles/litre in Surfactants and Interfacial Phenomena, Milton Rosen, Wiley 1978 (other literature reports lower Krafft temperatures);
sodium dodecyl sulphonate for which the same reference quotes a Krafft temperature of 38°C and a critical micelle concentration of approximately 10mMole/litre;
sodium di C6-C8 alkylsulphosuccinate having a Krafft temperature of 15-18° C;
sodium cocoyl isethionate (Elfan® AT 84G from Akzo Chemie) whose manufacturers state that it has a Krafft temperature of 26°C. Parris et al JAOCS 49 649 report a critical micelle concentration of approximately 6mMole/litre for the dodecyl component which predominates. This surfactant forms hexagonal liquid crystal phases (as well as lamella phases) on contact with water above the Krafft temperature. This isethionate was used in several different particle sizes which were obtained by grinding and sieving the commercial noodles of this surfactant.

### Example 1

Wiping articles prepared as above, using various surfactants, were tested by a procedure to determine the number of times they could be wet and squeezed out before becoming exhausted of surfactant. This test was carried out as follows. 25g of water (tap water of approximately 10° French hardness at a temperature of 35-40°C) was poured on to a wiping article which was then squeezed, thereby squeezing out approximately half the water from the article. The water squeezed out was poured into a 100ml measuring cylinder and shaken for 5 seconds. Any surfactant dissolved from the wiping article would cause foaming. A foam volume greater than the volume of liquid in the measuring cylinder after standing for two minutes was regarded as adequate foaming. The procedure was repeated until the observed foaming ceased to be adequate. The number of cycles of wetting and squeezing out in this fashion before foaming ceased to be adequate are given in the table below, which also states the surfactant employed and its particle size.

As can be seen from the table, with both sodium dodecyl sulphate and dialkylsulphosuccinate, which do not meet the requirements of this invention, the number of cycles before exhaustion was not greatly increased by increasing the amount of surfactant in the wiping article whereas with sodium cocoyl isethionate the number of cycles before exhaustion increased with increasing amounts of surfactant in the wiping article, indicating that the rate of dissolution of the surfactant was slower.

The particle size of the isethionate also had an effect: larger particles dissolving more slowly. With the largest particles of isethionate the rate of dissolution was so slow that 0.2g surfactant did not give adequate foaming at all. Even the higher loadings of the larger sizes gave poor foam on the first cycle of wetting and squeezing out.

For a preferred wiping article isethionate was used, applying 0.1g of particles smaller than 0.35mm and 0.4-0.9g of particles in the 0.5 to 1.0mm size range.

When the surfactant was sodium dodecyl sulphate the wiping articles appeared to be producing more foam than desired, and felt slimy, except when the amount of surfactant included in the wiping article was at the low (0.2g) level. This was also observed with the wiping articles having dialkylsulphosuccinate as surfactant. When sodium cocoyl isethionate was used as surfactant this over foaming and apparent slimy feel were less apparent than with the other two surfactants.

### Example 2

A comparison was made between wiping articles made by the above general procedure, using sodium dodecyl sulphate in one case and sodium dodecyl sulphonate in the other. Both surfactants were sieved before the articles were made, so that the surfactant particles had a size no greater than 0.5mm.

The release of surfactant from the articles was tested by the following procedure. 25g of water (approximately 10° French hardness) at a temperature of 25°C was poured on to a wiping article. The article was squeezed, thereby squeezing out approximately half the water from the article. This water was collected. The cycle of wetting the article, squeezing and collecting the expressed water was carried out repeatedly. The concentration of surfactant in samples of the expressed water was determined by titration with hyamine, which is a cationic surfactant. The extent of foaming was also noted. Results are set out in the following Table.

The results with sodium dodecyl sulphonate showed some experimental variation, notably in the concentrations in the water expressed on the second and eleventh cycles.

However, the results clearly show that sodium dodecyl sulphate, whose Krafft temperature is below the temperature of the water used in the test and which does not exist as a liquid crystal phase at the test temperature, gave excessive initial release of surfactant. By contrast, sodium dodecyl sulphonate has its Krafft point above the test temperature and the release of surfactant was retarded, avoiding initial overfoaming and giving adequate foaming for a greater number of cycles of wetting and squeezing.

### Example 3

Wiping articles were made by the above general procedure. The surfactant employed was sodium cocoyl isethionate having a particle size in the range from 0.5 to 1mm.

The release of surfactant was determined by the procedure of Example 2. This test was carried out twice, once using water at 25°C and once using water at 35°C. The results are set out in the following table.

With water at 25°C, just below the Krafft temperature, there was steady release of surfactant similar to the result with sodium dodecyl sulphonate in Example 2.

With water at 35°C, which is above the Krafft temperature, the release of surfactant from the wiping article is slightly faster than at 25°C. Nevertheless it is a steady release, manifestly different from the rapid release of dodecyl sulphate in Example 2, because the surfactant forms a liquid crystal phase at the test temperature.

### Example 4

Wiping articles were prepared using sodium cocoyl isethionate of various particle sizes as used in Example 1.

The release of surfactant on initial wetting was tested by the procedure used in Example 2. The test was carried out using water at 35°C. The concentration of surfactant in the water expressed after first wetting was determined and the results are as follows:

Thus use of a large particle size with a small amount of small particle size enables good foam on the first cycle of wetting and squeezing as well as achieving retarded release.

## Claims

1. A substantially dry-to-the-touch wiping article which is suitable for use in cleaning soiled surfaces in the presence of water,
the article comprising first and second substrate layers with surfactant in solid form sandwiched between them,
characterised in that the surfactant
i) forms a liquid crystalline phase in contact with water at temperatures above its Krafft temperature and up to at least 30°C, and/or
ii) has a Krafft temperature above 20°C.

2. An article according to claim 1 wherein the pure surfactant is capable of existing in dry particulate form at 20°C.

3. An article according to any one of the preceding claims wherein the surfactant forms a hexagonal or cubic liquid crystalline phase on contact with water at temperatures above its Krafft temperature and up to at least 35°C.

4. An article according to claim 3 wherein the surfactant forms the liquid crystalline phase at temperatures up to at least 50°C

5. An article according to any one of the preceding claims wherein the surfactant is a salt of an acyl isethionate wherein the acyl group contains from 8 to 22 carbon atoms, the salt being formed by a solubilising cation.

6. An article according to claim 5 wherein the fatty acyl group is coconut acyl.

7. An article according to any one of the preceding claims wherein the surfactant has a critical micelle concentration of at least 2mMole/litre.

8. An article according to claim 7 wherein the critical micelle concentration is at least 4mMole/litre.

## Patentansprüche

1. Ein im wesentlichen Trocken-zu-der-Berührung-Wischgegenstand, der geeignet für eine Verwendung zum Reinigen verschmutzter Oberflächen in Gegenwart von Wasser ist,
wobei der Gegenstand erste und zweite Substrat-Schichten mit in Sandwichform dazwischen gelagertem Surfactant in fester Form umfaßt,
**dadurch gekennzeichnet,** daß das Surfactant
i) eine flüssigkristalline Phase in Kontakt mit Wasser bei Temperaturen oberhalb seiner Krafft-Temperatur und bis zu zumindest 30°C bildet, und/oder
ii) eine Krafft-Temperatur von über 20°C aufweist.

2. Gegenstand nach Anspruch 1, **dadurch gekennzeichnet,** daß das reine Surfactant fähig ist, in trockener Teilchenform bei 20°C vorhanden zu sein.

3. Gegenstand nach irgendeinem der vorhergehenden Ansprüche, **dadurch gekennzeichnet,** daß das Surfactant eine hexagonale oder kubische flüssigkristalline Phase beim Kontakt mit Wasser bei Temperaturen oberhalb seiner Krafft-Temperatur und bis zu zumindest 35°C ausbildet.

4. Gegenstand nach Anspruch 3, **dadurch gekennzeichnet,** daß das Surfactant die flüssigkristalline Phase bei Temperaturen bis zu zumindest 50°C ausbildet.

5. Gegenstand nach irgendeinem der vorhergehenden Ansprüche, **dadurch gekennzeichnet,** daß das Surfactant ein Salz eines Acylisethionats ist, worin die Acylgruppe von 8 bis 22 Kohlenstoffatome enthält, wobei das Salz durch ein solubilisierendes Kation gebildet wird.

6. Gegenstand nach Anspruch 5, **dadurch gekennzeichnet,** daß die Fettsäureacylgruppe Kokosnußacyl ist.

7. Gegenstand nach irgendeinem der vorhergehenden Ansprüche, **dadurch gekennzeichnet,** daß das Surfactant eine kritische Micell-Konzentration von zumindest 2 mMol/ℓ aufweist.

8. Gegenstand nach Anspruch 7, **dadurch gekennzeichnet,** daß die kritische Micell-Konzentration zumindest 4 mMol/ℓ beträgt.

## Revendications

1. Article d'essuyage sensiblement sec au toucher, qui convient pour utilisation dans le nettoyage de surfaces salies en présence d'eau,
l'article comprenant une première et une seconde couches de substrat entre lesquelles un tensio-actif solide est pris en sandwich,
caractérisé en ce que le tensio-actif
(i) forme une phase cristalline liquide en contact avec l'eau à des températures au dessus de sa température Krafft et jusqu'à au moins 30°C, et/ou
(ii) présente une température Krafft au dessus de 20°C.

2. Article selon la revendication 1, dans lequel le tensio-actif pur peut exister sous une forme particulaire sèche à 20°C.

3. Article selon la revendication 1 ou 2, dans lequel le tensio-actif forme une phase cristalline liquide hexagonale ou cubique lors de son contact avec l'eau à des températures au dessus de la température Krafft et jusqu'à environ 35°C.

4. Article selon la revendication 3, dans lequel le tensio-actif forme la phase cristalline liquide à des températures allant jusqu'à au moins 50°C.

5. Article selon l'une quelconque des revendications précédentes, dans lequel le tensio-actif est un sel d'un acyl-iséthionate dont le radical acyle contient de 8 à 22 atomes de carbone, le sel étant formé par un cation solubilisant.

6. Article selon la revendication 5, dans lequel le groupe acyle gras est le coprah-acyle.

7. Article selon l'une quelconque des revendications précédentes, dans lequel le tensio-actif présente une concentration critique de micelles d'au moins 2 mmoles/litre.

8. Article selon la revendication 7, dans lequel la concentration critique de micelles est d'au moins 4 mmoles/litre.
